

## UNITED STATES PATENT OFFICE

CHARLES D. PARKS, OF DANBURY, CONNECTICUT

## ART OF FELTING

No Drawing. Application filed April 8, 1925, Serial No. 21,999. Renewed February 14, 1930.

This invention relates to the art of felting and, with regard to its more specific features, to the art of making felt such as is used in the manufacture of felt hats.

- 5 One of the objects of this invention is to provide a simple and practical art of making felt from fur or the like and, moreover, to provide an art of this nature which may be readily and inexpensively carried on in practice and in a manner that will avoid endangering the health of the workmen carrying on the art. Another object is to provide 10 an art of felt manufacture which may be carried on efficiently and in a manner free 15 from the defects and disadvantages characteristic of felt manufacture as it has been carried on for many years in the past and in the course of which fur treated with mercuric nitrate has been universally employed. 20 Another object of this invention is to provide an art of the above-mentioned character which may be readily and inexpensively carried into or incorporated in the manufacture of felt hats. Other objects will be in 25 part obvious or in part pointed out herein-after.

The invention accordingly consists in the several steps and relation and order of each of the same to one or more of the others, all 30 as will be illustratively described herein, and the scope of the application of which will be indicated in the following claims.

As conducive to a clearer understanding of this invention, it may at this point be noted 35 that in the manufacture of felt from fur or similar fibrous animal products, as is carried on in the manufacture of hats, for example, it has been the practice for many years in the past to use fur which has been 40 prepared for felting by a carroting process in which mercury nitrate, a compound form of mercury and nitric acid, is applied to the fur or fur fibers. While fur thus prepared, that is by the mercury nitrate treatment, 45 produces a good grade of ultimate felt, the fur itself is impregnated with this mercury compound and is hence poisonous; the carroting or initial treatment of the fur to give it felting properties involves the 50 handling not only of this poisonous com-

pound but also of the resultant treated fur, and thus the health of the operatives employed in this process is greatly jeopardized. But in the subsequent processes through 55 which the fur is placed, as in the felting processes and the earlier steps in the course of the manufacture of a hat body, this poisonous and mercury-bearing fur and resultant felt carries into these steps or processes the same mercury compound and causes great 60 injury, due to mercurial poison, to the workmen employed. One of the dominant aims of this invention is to provide an art of felt manufacture wherein such serious consequences and disadvantages as are briefly 65 pointed out hereinabove may be avoided and eliminated in a manner at once simple and inexpensive as well as thoroughly practical.

In my Patent No. 1,507,892, dated September 9, 1924, I have disclosed an art of treating fur or similar material to give it felting properties and in the course of which art the fur fibers are treated with a solution in which is included an oxidizing agent, such as 70 hydrogen peroxide, for example, and a cleansing agent, such as sodium hydroxide, for example, and with the resultant fur described in the said patent and as a result of the process therein described I am enabled to produce a resultant felt of excellent qualities, thoroughly practical and free from the defects 75 whereby the operatives are subjected to mercurial poisoning. I have discovered, however, that the elimination of mercurial poisoning, while at the same time attaining 80 thoroughly practical results, may be achieved by continuing the treatment of the fur fibers in the course of the felting operations with a material capable of a peculiar interaction 85 with a simpler and less expensive carroting material than is disclosed in my above-mentioned patent and in my Patent No. 1,507,891.

Considering now certain features of my invention, it might first be pointed out that the 90 formation of felt from fur or the like is achieved by the action of the individual fibers in interlocking or "interfelting" one with another, but because the natural fur fibers carry a certain grease, wax or gummy substance and other foreign materials, the latter 95

55

60

65

70

75

80

85

90

95

100

substances or materials prevent this interlocking action, doubtless because the many scales or barbs which appear on the surface of the individual fibers are precluded thereby from taking part in this interlocking action. To achieve a thoroughly practical felt these barbs or scales must be made available to take part in the interlocking action, and hence the wax, which term will hereinafter be used to designate the substances or materials that appear naturally upon the surfaces of the individual fibers, must be either removed or so treated that it may be in subsequent operations or steps dissolved or washed out.

In accordance with my invention, I first form a solution with a hydroxide, preferably a hydroxide of an alkali metal and preferably sodium hydroxide or potassium hydroxide, the latter being readily available commercially, and with water form such a solution that it will have a strength of between 1° Baumé and 10° Baumé, though better results I have found are more readily assured if the strength of the solution is within the limits of 2½° Baumé to 7° Baumé. With this solution I treat the fur, preferably while it is still upon the skin, as by brushing the solution to the fur fibers on the skin. The fur is then dried, whereupon it is removed from the skin. The resultant fur fibers will thus bear and carry a material or substance which is the result of the action of the hydroxide upon the wax on the fur fibers, and if such a fur, as has already been in the prior art proposed, is subjected to the usual felting steps or processes, it will be found to have merely a tendency to interlock or felt but will be devoid of a felting or interlocking action which will be characterized by the mechanical strength and integrity of structure necessary for it even to withstand succeeding steps in the manufacture of a hat body, for example. Such a weakness mechanically makes it impracticable to work the so-called fabric up into its successive stages in the course of the manufacture of the hat body and ultimate hat, and another defect which such a fur has been found to have resides in the fact that whatever tendency to felt or interlock that it has is not uniform. This latter defect results in a fabric which is uneven and non-uniform both as to thickness and as to mechanical strength, and these latter defects are emphasized as the hat body undergoes further succeeding steps.

The use of a hydroxide such as sodium hydroxide or potassium hydroxide in the initial step of preparing the fur fibers for felting embodies certain advantages, some of which have hereinbefore been pointed out, and in accordance with my invention I make it possible to achieve these advantages while avoiding the defects just above pointed out. The fur fibers, thus carrying the product which results from the interaction of the hydroxide

upon the wax, are thereupon "formed" into a sheet or layer, as by blowing the fur fibers onto a perforated support, which support in the case of the manufacture of hat bodies is generally of conical shape. The resulting conically shaped hat body is termed a "bat", and immediately after its formation as above described I treat the bat, as by immersion or spraying, with water which has been acidified. Thus I treat it in this manner with water to which an acid has been added in the proportion of about sixteen ounces of acid to three hundred gallons of water. Any suitable acid may be employed. I prefer in practice to employ formic acid. By way of illustration, I may use acetic acid to bring about the acidification and, in certain instances depending upon the character of the fur, I may employ sulphuric acid.

The bat or hat body is then "wet down" and "hardened", in the course of which the bat is kneaded, generally manually, while at the same time making frequent applications thereto of water at an appropriate temperature. In accordance with my invention, however, I carry on the wetting down and hardening steps, in the course of which the fibers may be considered as being given an initial interlocking or interfelting, by making, during the steps, frequent applications of a solution having an acid reaction. This solution is preferably water to which has been added an acid, preferably formic acid as above described, and this solution may conveniently be made in the proportion of from two to four ounces of acid for each fifteen gallons of water.

After the hat has been hardened and the interfelting or interlocking of the fur fibers initiated, the hat body or bat is "sized". In this operation the bat is vigorously kneaded, and, in accordance with my invention, I apply frequently to the hat body or bat as the latter is kneaded a hot solution having an acidic reaction; this solution is preferably water at an appropriate temperature to which I have added an acid, preferably formic acid, as hereinbefore pointed out in connection with prior steps of the felting operation, and the degree of acid employed during the sizing of the bat or hat body is substantially like that employed during the step of hardening. During the sizing, the bat or hat body is progressively shrunk due to the fact that the interlocking action of the fur fibers is made so complete that the resultant fabric is of great mechanical strength and tightness. The felting of the fur fibers is thus substantially completed and the fabric or hat body is ready to be subjected to further steps as in the manufacture of felt hats.

The action of the acid in the above-described successive steps involved in the felting appears to be one which, in the course of

these steps of felting, completes the preparation of the individual fur fibers for effective and uniform interlocking or interfelt action. The product carried by the fur fibers and resulting from the interaction of the hydroxide with the wax on the fur fibers is an impediment to achieving practical felting, but the interaction of the acid solution or solutions characteristic of certain of the subsequent steps of felting in accordance with my invention removes this impediment, the acid in turn interacting, and, perhaps by gradual neutralization of the above-mentioned resultant product, probably largely alkaline, makes possible the ultimate and complete removal of this product or its reduction to a soluble state; thus the barbs or scales, even if only partially placed in condition to be partially available in the course of the initial treatment of the fur fibers by hydroxide, are made progressively more available as the latter felting steps are carried on, and finally made completely available to bring about an ultimate felt capable of meeting the requirements of practice. Thus it will be seen that, by continuing the treatment of the fur fibers or the wax thereon during the felting operation, a thoroughly efficient interlocking may be achieved even though the initial step of treating the fur fibers or the wax thereon, as by the hydroxide, leaves the fur fibers in a condition of but imperfect felting properties.

While good results may be achieved in applying the acidified solution only during one of the steps of felting treatment hereinbefore described, thus to permit the substantial completion of the preparation of the fur fibers for felting, yet I prefer to carry on the application of the acidified solution throughout each of the several steps as hereinbefore described in order thus to compensate for the progressive diminution of the acid content in any one step due to the gradual neutralization of the acid by the alkaline component of the product carried by the fur fibers; though it will be understood that the acid content may be maintained within the desired limits by replenishment of the acid as the latter is progressively neutralized.

As the art herein described might be varied in various parts all without departing from the scope of the invention, it is to be understood that all matter herein set forth is to be interpreted as illustrative and not in a limiting sense.

I claim as my invention:

1. The herein described art of felting which consists in treating fur or the like with a solution of a hydroxide of an alkali metal adapted to react with the wax on the fibers thereof and give the latter felting tendencies, drying the fur, forming a fabric out of the fur, felting the fibers of the fabric together, and in treating the fibers of the fabric during

the felting operation with a solution having an acid reaction to complete the preparation of the fibers for felting.

2. The herein described art of felting which consists in treating fur or the like with a solution of a hydroxide of an alkali metal adapted to react with the wax on the fibers thereof to give the latter felting tendencies, drying the fur, forming a fabric out of the fur, treating the fibers of the fabric with a solution adapted to complete the preparation of the fibers for felting, and felting the fibers of the fabric together. 70 75

3. The herein described art of felting which consists in treating fur or the like with a solution of a hydroxide of an alkali metal adapted to react with the wax on the fibers thereof to give the latter felting tendencies, drying the fur, forming a fabric out of the fur, treating the fibers of the fabric with a solution having an acidic reaction and adapted to complete the preparation of the fibers for felting, and felting the fibers of the fabric together. 80 85

4. The herein described art of felting which consists in treating fur or the like with a solution adapted to react with the wax on the fibers thereof and to partially prepare the fibers for felting, forming a fabric out of the fibers thus treated, treating the fabric with a solution adapted to complete the preparation for felting of the fibers thereof, and felting the fibers of the fabric together. 90 95

5. The herein described art of felting which consists in treating fur or the like with an alkaline solution adapted to react with the wax on the fibers thereof and to give the latter a felting tendency, forming a fabric out of the fur fibers thus treated, treating the fibers of the fabric with a solution having an acidic reaction to complete the preparation of the fibers for felting, and felting the fibers of the fabric together. 100 105

6. The herein described art of felting which consists in forming a fabric out of fur or the like having upon the fibers thereof a product resulting from the reaction of the natural wax thereon with an alkaline solution which partially prepares the fibers for felting, treating the fabric with a solution adapted to attack the product on the fibers thereof to improve the felting properties of the fibers, and felting the fibers of the fabric together. 110 115

7. The herein described art of felting which consists in forming a fabric out of fur or the like having upon the fibers thereof a product resulting from the reaction of the natural wax thereon with an alkaline solution which partially prepares the fibers for felting, and felting the fibers of the fabric together while applying thereto an acid solution adapted to attack the product carried by the fibers to improve the felting properties of the fibers. 120 125 130

8. The herein described art of felting which consists in forming a fabric out of fur or the like having upon the fibers thereof a product resulting from the reaction with the natural wax thereon of an alkaline solution which partially prepares the fibers for felting, treating the fabric with an aqueous solution of formic acid to improve the felting capacity of the fibers, and felting the fibers of the fabric together.

9. The herein described art of felting which consists in forming a bat out of fur or the like having upon the fibers thereof a product resulting from the reaction with the natural wax thereon of an alkaline solution which partially prepares the fibers for felting, treating the bat with a solution having an acid reaction and adapted to react with the product on the fibers to improve the felting properties of the fibers, hardening the bat, and thereupon shrinking the bat to complete the interfelting of the fibers thereof.

10. The herein described art of felting which consists in forming a bat out of fur or the like having upon the fibers thereof a product resulting from the reaction with the natural wax thereon of an alkaline solution which partially prepares the fibers for felting, hardening the resultant bat while applying thereto a solution having an acid reaction and adapted to react with the product on the fibers to improve the felting properties of the fibers, and sizing the bat.

11. The herein described art of felting which consists in forming a bat out of fur or the like having upon the fibers thereof a product resulting from the reaction with the natural wax thereon of an alkaline solution which partially prepares the fibers for felting, hardening the bat, and shrinking the hardened bat while applying thereto a solution adapted to react with the product on the fibers thereof to improve the felting properties of the fibers.

12. In testimony whereof, I have signed my name to this specification this 4th day of April, 1925.

CHARLES D. PARKS.

50

55

60

65